

E. J. GUAY,  
COMPOSITION FOR ARTIFICIAL BUILDING MATERIAL, TRIMMINGS, &c.  
APPLICATION FILED MAY 6, 1911.

1,188,759.

Patented June 27, 1916.

Fig. 1.



Fig. 2.



Witnesses:

William M. Lyon  
Ernest C. Schaum

Inventor,

Emile J. Guay.  
By John A. McMannus,  
Atty.

# UNITED STATES PATENT OFFICE.

EMILE J. GUAY, OF SWAMPSOFT, MASSACHUSETTS, ASSIGNOR TO GENERAL CERAMIC MANUFACTURING COMPANY, A CORPORATION OF MAINE.

## COMPOSITION FOR ARTIFICIAL BUILDING MATERIAL, TRIMMINGS, &c.

1,188,759.

Specification of Letters Patent. Patented June 27, 1916.

Application filed May 6, 1911. Serial No. 625,454.

To all whom it may concern:

Be it known that I, EMILE J. GUAY, a citizen of the United States, residing at Swampscott, county of Essex, and State of 5 Massachusetts, have invented new and useful Improvements in Composition for Artificial Building Material, Trimmings, &c.

This material is especially applicable to the manufacture of poles for telegraph, telephone and street lighting purposes, etc., which shall be durable, against the ravages of weather and other injurious effects to which wooden poles are subjected, and also to provide a process which enables this 10 15 position to be commercially handled to advantage.

Figure 1 represents a car of sand lime blocks in the steaming or indurating chamber during that part of the process in which 20 the blocks of my invention are being hardened or indurated. Fig. 2 represents a car upon which is mounted a block of building material, one-half of which block is made by the protected process and the other half 25 by the unprotected process.

Referring more particularly to Fig. 1, 1 represents a suitable steam chamber into which is led a pipe 2, for conveying steam under suitable pressure, say 150 pounds to 30 the square inch into said chamber, and at a temperature corresponding to this pressure of about 360 degrees F. 3, 3', represent suitable angle irons or rails upon which angle irons or rails in the chamber 1, is 35 mounted a car 4, supported by the wheels 5, the latter in turn being suitably mounted in supports or bearings depending from the bottom of the car 4. 6 6', etc., represent in dotted lines blocks of my improved material 40 mounted upon the car 4, these blocks being covered with sand or other inert material 7 in such manner as to be protected from the direct action of the steam. The right hand end of the car, however, is shown in section 45 in order to illustrate more clearly the exact arrangement of the blocks and to remove the obscurity of the view caused by the sand. 8 8' represent sides composed of metal or other suitable material which merely serve 50 as retaining walls for the blocks and sand.

Referring now more particularly to Fig. 2, upon the car 4, is mounted a large block of building material 9, the left hand half of which is protected by a covering of sand 7. 55 The right hand portion 10, of the block is

unprotected and being made of the same fineness of division of mixture and in exactly the same manner all through the process with the exception that it is not covered with sand during the induration, it will be 60 found to disclose various small cracks such as illustrated at 11, 12, 13, 14, etc., and to disclose the general characteristics of a poor piece of building material.

My invention consists in making blocks of 65 a mixture of silica and hydrated lime in the following proportions: silica 85% to 95%, hydrated lime 5% to 15%, the preferable mixture, however, being silica 88% to 90%, hydrated lime 10% to 12%, the effective 70 binder, hydrous silicate of lime, resulting from this mixture being uniformly distributed throughout the mass. A certain percentage of sand and lime in the mixture chemically unite, and this chemical combination results in the production of hydrous silicate of lime which forms a binder for the remaining portion of sand and lime, which is not chemically combined. In other words, part of the original mass of sand 80 and lime becomes chemically united, while any portion which is not so chemically united becomes bound together by the chemically united portions. In the manufacture of poles, window trimmings, etc., especially, it is preferable to have the material mixed wet in order that it may be satisfactorily handled and worked or tamped in the mold. The difficulty about mixing it wet, however, is that the composition cannot be 85 indurated that way, as in the absence of a protecting blanket, the indurating fluid has a too rapid and direct action (apparently a chemical action) on the surface of the block, causing said surface to warp, crack, or 90 otherwise be distorted. Therefore, it has been found that, to avoid this difficulty, by embedding the block in an inert or porous material such as sand, the deleterious action of the indurating fluid is obviated. In the 100 application of my invention steam is the preferable fluid used for indurating.

After the block has been protected as above outlined it is subjected to the hardening or indurating process by the action 105 thereon of steam under suitable pressure; by a pressure say, of about 150 lbs. to the square inch.

Applicant's theory of the action resulting from this treatment is as follows: The pro- 110

tection for the block prevents the outside surface from shrinking, and, therefore, the water in the block, when it assimilates the lime and expands, is not limited in its chemical action and expansion to more confined limits resulting in the warping, cracking and distortion of the block. This process, therefore, results in a better finished product, as the more water that can be introduced into the mixture without causing the cracking referred to the better and stronger will be the artificial composition produced, the proportion of the crushing strength thus attained depending upon the amount of water which can be satisfactorily assimilated; and it has been found that from 15% to 18% water can be thus assimilated in the protected block as against 7% or 8% in the case of an unprotected block of a given initial cubical capacity.

When the mixture of sand and lime is taken from the mixer a considerable amount of water is added thereto (or an excess of water may be added during the mixing operation) whence the material is placed in a mold and subjected in a press to a pressure of from 2000 to 3000 lbs. per square inch; or in the forming of large blocks or pieces the block may be formed in an ordinary mold and tamped therein. The blocks are subsequently placed on a metal floor on a flat car or on a floor coated with sand, said blocks being laid up in a fashion somewhat like a pyramidal pile in receding layers. They are then covered with sand until they are completely buried in it and in such manner that the sand can get into all the interstices or spaces between the blocks (the blocks in this case usually being bricks in the stage of manufacturing prior to the hardening or indurating process); or a retainer may be formed as previously referred to, by protecting the sides of the pile by abutting side pieces of metal. The car is then wheeled on a track into a long oven into which steam is led and maintained at about 150 lbs. pressure to the square inch. The door of the oven is then closed or sealed. When the bricks are taken out of this oven after remaining therein subject to the action of the steam as above-mentioned for from seven to twenty hours, varying in accordance with the size of the piece or pieces being indurated, the finished product is found by test to withstand a crushing stress of about 10,000 lbs. pressure to the square inch, whereas the best product which applicant has been enabled to obtain by open baked methods will withstand a compression stress of only about 3000 lbs. to the square inch. In the latter methods it is not possible to assimilate enough water, because when the bricks are indurated in the open, or unprotected from the direct action of the steam the result is a greater amount of uncom-

bined hydrated lime in the finished product. If the bricks are indurated open or unprotected, and wet, the surface will crack; if indurated open, and dry, the resultant brick is not strong enough to use in high building structures; but when indurated wet and protected it gives a very strong product. Experiment has shown that with a given pressure of press and a given percentage of water that the product will crack when made by the unprotected process, but that with the same pressure and same percentage of water a brick made by the protected process will not crack. The degree of wetness varies with the fineness of grain of the materials; if one starts with 7% free water the brick will crack upon addition of 3% more unless it is protected during induration, as hereinafter described.

When the mixture containing a comparatively large amount of water, and molded into the form or shape of the finished article, is indurated in a manner to protect it from the indurating fluid as heretofore described, it is found that the resultant product is from seven to ten per cent. heavier than when a similar mixture is molded and indurated in an unprotected block. Applicant believes that what takes place is that when the mixture containing a comparatively large amount of water is used in the manufacture of artificial building materials the chemical action between the lime and the sand is greatly enhanced, resulting, of course, in the formation of a much larger percentage of the hydrous silicate of lime, which is generally considered as the binder in such matters. There is, therefore, left less uncombined hydrated lime which acts only as a poor filler occupying space which is more desirably filled by the hydrous compound or by silica.

Several very important incidents of the treatment described result from the equable application of the heat furnished by the steam, as it enforces a slow, gradual and uniform distribution of heat throughout the body treated; therefore the grains of the compound are not suddenly torn apart to accommodate the absorption and assimilation of more water, but the process takes place slowly and gradually similar to the growth of a crystal with an analogous increase of strength in its structure; similarly the body after treatment can only slowly cool and something akin to the annealing of a metal takes place toughening it and preventing fissures. Therefore no seams, cracks or weakened lines are found in the indurated product. Another very important incident is that the steam being moist prevents loss of water in the very wet mass; the water it contains from the initial mixing cannot evaporate and under the slow heating the calcium silicate formed gradu-

ally builds up in the pores and around the grains somewhat after the manner nature follows in forming crystalline structures so that the grains are welded in all directions by a rocky bond of enormous strength. The annealing action and the prevention of loss of water I consider the distinguishing features of my process. It takes place only at a critical temperature range, since if steam at 200 lbs. be applied the product will be weak and not in the same class with the product made under the conditions herein described. The conditions described seem to limit the ingress of heat and moisture to the molded product in the best way to insure a product of maximum strength free from cracks, and therefore the most desirable for use in industrial arts.

Another way this may be put is that by the assimilation of more water the small particles of binding material are allowed to flow more freely and thus find entrance into whatever interstices may exist, thus more thoroughly impregnating the product with the binding material. Another thing, on account of this more complete assimilation of water during the process of manufacture, after the brick is finished and hardened it will have a low affinity for extraneous water or moisture, and will, therefore, be more frost-proof, increasing in weight not more than 4% after setting in water for more than 10 hours, whereas in the case of the best products known to applicant resulting from processes practised by other than his invention the increase in weight by similar test is in the neighborhood of, or more than, twice this percentage. When seven or eight per cent. of lime is used in the protected block process the product is found to have twice or three times the compression strength of that of the unprotected block process using the same percentage of lime.

It is therefore evident from the foregoing that I have developed a process which is novel, simple, effective, and one which enables the mixture to assimilate more water, thereby adding materially to the density, homogeneity, compression and tensile strengths and general improved characteristics of sand-lime bricks or products.

What I claim as new and desire to secure by Letters Patent of the United States is:

1. The process of manufacturing composition for artificial building materials which consists in mixing materials capable of chemically combining in a moist state and under heat and pressure, making a wet mixture of the said materials containing an excess of free water, molding the materials under pressure, and heating the mixture under conditions which prevent loss of water.

2. The process of manufacturing the composition herein described consisting of mak-

ing a wet mixture of silica and hydrated lime in substantially the proportions of silica 85% to 95%, and hydrated lime 5% to 15%, forming said mixture under pressure into an article of the desired shape, enveloping 70 said article completely in suitable material in such manner as to protect it from the direct action of steam during the indurating process, and finally hardening or indurating the article by subjecting it to the action of 75 steam under pressure of approximately 150 pounds.

3. The process of manufacturing the composition herein described consisting of making a wet mixture of silica 85% to 95% 80 and hydrated lime 5% to 15%, molding said mixture under pressure into a block of the desired form, placing said block in a retainer, protecting all exposed surfaces of the block from the direct action of steam during 85 the indurating process by completely covering them with inert material permitting slow and equable heat access, and finally indurating the block by subjecting it to the action of steam under pressure of approximately 90 150 pounds.

4. The process of manufacturing a sand lime compound consisting in making a wet mixture of sand and hydrated lime with the sand in large excess, molding the mixture, 95 heating it under steam at 150 pounds pressure, protecting the molded article with a covering adapted to retard the ingress of heat and rendering it equable throughout the mass and insuring access of steam uniformly over the entire mass.

5. The process of manufacturing a sand-lime composition consisting of making a wet mixture of silica and lime in substantially the proportions of silica 85% to 95% and 105 lime 5% to 15%, molding said mixture under pressure into blocks of the desired form, protecting all exposed surfaces of the block completely from the direct action of the steam during the indurating process for 110 the purpose of assimilating the maximum amount of water which can be assimilated within such protected block, and finally indurating the block by the action of steam at a temperature corresponding to a pressure 115 of 150 pounds and upward.

6. The process of manufacturing a sand lime composition of great density and compression strength, consisting in making a wet mixture of silica and lime of the preferable proportions of silica 88 to 90 per cent. and hydrated lime 10 to 12 per cent., molding it into bricks of the desired form, protecting the surfaces completely from the subsequent indurating agent, and indurating by action of steam under a pressure of approximately 150 pounds applied outside the protecting medium in an indurating oven, and slowly heating them while preventing loss of water.

7. The process of manufacturing artificial stone consisting of making a wet mixture of silica and lime in substantially the proportions of silica 88% to 90% and hydrated lime 10% to 12%, molding bricks of the mixture under pressure, protecting the bricks from the direct action of the steam during the indurating process, and finally indurating the bricks in an indurating oven 10 in which steam is confined under a pressure of approximately 150 pounds.

8. The process of manufacturing composition for building materials which consists in mixing materials capable of chemically combining in a moist state and under heat and pressure, making a wet mixture of the said materials, molding the materials into the desired form, completely embedding the molded article in a porous heat retarding material, and subjecting the molded product to a heated fluid and under a pressure of at least 150 pounds and upward acting on its entire surface through said porous material.

9. The process of manufacturing artificial building material consisting in mixing sand and lime with a large excess of water, exposing to slowly acting moist heat, while preventing loss of water by evaporation and thereby slowly indurating the mixture by

cementing its particles into a solid mass of fine texture.

10. The process of manufacturing composition for building materials capable of chemically combining in a moist state and under heat and pressure, which consists in 35 making a mixture of said materials in suitable proportions and with an excess of water amounting to wetness, molding the mixture into the desired shape, protecting the molded article from the direct action of steam 40 under pressure used as an indurating fluid by interposing a body of inert porous material between the steam and the molded article throughout its entire surface for the purpose of increasing the effective amount 45 of water content in the mixture to secure the formation of the maximum amount of hydrous silicate of lime possible to be formed therein, and finally hardening the molded article by subjecting it to a heated fluid such 50 as steam under suitable pressure acting through the inert materials.

In witness whereof, I have hereunto set my hand this 4th day of May, 1911.

EMILE J. GUAY.

Witnesses:

FRANK G. HATTIE,  
JOHN A. McMANUS, Jr.